

## UNITED STATES PATENT OFFICE.

ARTHUR C. ZIMMERMAN, OF DAYTON, OHIO.

## TREATMENT OF MAGNESIUM AND MAGNESIUM ALLOYS TO INHIBIT CORROSION.

No Drawing.

Application filed October 31, 1924. Serial No. 747,128.

REISSUED

This invention relates to the treatment of magnesium and magnesium alloys, so as to inhibit or prevent corrosion, to which metals of this type are quite susceptible. 5 I have discovered that if an article made of magnesium or magnesium alloys in which magnesium is present as the major constituent, are subjected to the action of a dilute solution of phosphoric acid, boric acid, 10 borax or other borates of the alkali metals, a coating or impregnation of phosphate, borate, or other compound of magnesium likely to form under the treatment, is produced. It is also desirable to have present 15 in the treating solution, an oxidizing salt such as manganese dioxide. As an example of a treatment which affords ample protection, the following is submitted: The material is immersed in a .75 per cent by volume 20 solution of phosphoric acid, containing about 1 ounce of manganese dioxide per gallon of solution. At the time the metal is immersed the solution should be heated to about 200° Fahrenheit, and this temperature 25 maintained after the immersion of the metal, which remains immersed until a continuous coating or impregnation of the dark gray colored compound of magnesium is formed, or until practically all gas ceases to 30 be evolved from this solution. Usually about one and one-half hours are sufficient for the complete treatment of the metal in the solution.

The metal is then removed from the solution and washed with water. After the 35 washing with water, it is heat-treated by placing it in an oven. After baking for a short time, sufficiently to thoroughly dry and stabilize the coating, it is removed and 40 cooled to room temperature. Subsequently a coating or coatings of paint, enamel or lacquer, or combinations thereof are applied, depending upon the results desired. It has been found that, for inhibiting corrosion 45 when exposed to the atmosphere, salt water, benzol or gasoline, two coatings of bakelite lacquer serve the purpose excellently as a finishing coating metal.

Although the protection afforded by subsequent heat treating and painting is greatly improved thereby, these two steps are not absolutely essential in the treatment of the metal. Very good results are obtained by 50 merely subjecting the metal to the action of the phosphoric acid, boric acid or borax as

the case may be, and merely washing or drying the treated metal.

It is essential that the solution of acid used be sufficiently weak so as to prevent too rapid action on the metal. In case the acid 60 is stronger than it should be, the acid eats into the metal so rapidly that the scales or protective coating is loosened and does not rigidly adhere to the product. It has been found that a  $\frac{1}{2}$  to a 1 per cent solution of 65 phosphoric acid is most desirable, but if the time is increased considerably, a weaker solution than  $\frac{1}{2}$  to 1 per cent may be used. Similarly it is possible to use more than a 1 per cent solution of phosphoric acid for a 70 shorter period of time, although in such case the protective coating is not quite as integral as the coating which would be produced more slowly.

When boric acid is used in place of phosphoric acid as the treating acid, the solution should be slightly stronger than 1 per cent, as the boric acid is not quite so active an agent in attacking magnesium. Less than a 5 per cent solution however should be used. 80 In the case of borax, it has been found that less than a 5 per cent solution should be used for the best results, but this salt also may be slightly stronger than the solution of phosphoric acid used.

The salts formed on the surface of the magnesium article treated are of an insoluble medium and are quite stable and serve to adequately protect the material beneath it. They also form a surface to which the paint 90 or lacquer may be effectively applied.

I claim:

1. The method of treating magnesium and magnesium base alloys to inhibit corrosion, comprising treating the metal with a solution of not more than five percent phosphoric acid, containing from one-tenth to ten ounces manganese dioxide per gallon of solution for about one and one-half hours.

2. The method of treating magnesium and magnesium base alloys to inhibit corrosion, comprising treating the metal with a solution of not more than five percent phosphoric acid, for about one and one-half hours at a temperature of about 200° Fahrenheit in the presence of from one-tenth to ten ounces manganese dioxide per gallon of solution.

3. The method of treating magnesium and magnesium base alloys to inhibit corrosion against natural and prepared agencies, com-

85

75

80

85

90

95

100

105

110

prising treating the metal with a solution of not more than five percent phosphoric acid, until a coating and impregnation of a magnesium phosphate is formed on the surface of the metal and subsequently drying the treated metal and coating with paint or lacquer.

4. The method of treating magnesium articles comprising treating the article in a water solution of less than 5 per cent of phosphoric acid, for about one and one-half hours at about 200° Fahrenheit in the pres-

ence of from one-tenth to ten ounces manganese dioxide per gallon of solution and subsequently drying the article.

5. The method of treating magnesium and magnesium base alloys to inhibit corrosion which consists of treating the metal with a solution of phosphoric acid until a protective coating of magnesium phosphate is formed on the surface of the metal.

In testimony whereof I affix my signature.

ARTHUR C. ZIMMERMAN.